

## UNITED STATES PATENT OFFICE

GEORGE A. RICHTER, OF BERLIN, NEW HAMPSHIRE, ASSIGNOR TO BROWN COMPANY, OF BERLIN, NEW HAMPSHIRE, A CORPORATION OF MAINE

## PULP REFINING AND BLEACHING PROCESS

No Drawing.

Application filed May 6, 1927. Serial No. 189,461.

This invention relates to the refining and bleaching of cellulose pulp, and has for its object the production of a product bleached substantially to ultimate whiteness and possessing certain optimum physical and chemical characteristics.

The usual bleaching of cellulose pulp effects both physical and chemical injury upon the fiber, the extent of such injury being determinable by physical characteristics such as tear resistance, and chemical characteristics such as copper number. Such injury may be materially reduced if the pulp is subjected to a distinctly alkaline bleaching treatment, as disclosed in application, Serial No. 716,153, filed May 27, 1924, by Milton O. Schur and myself, but even in such latter case the fiber is sometimes injured, particularly when the pulp is of a refractory nature and hence necessitates a relatively large amount of bleach to reach substantially ultimate whiteness. I have now found that injury to the fiber may be minimized, if in lieu of bleaching pulp to completion by one distinctly alkaline bleaching treatment, such pulp is subjected to a series of such treatments, preferably with alternating washings.

Such bleaching procedure finds especial utility in a process of refining raw wood pulp, and more particularly alkaline-digested pulps such as kraft and soda pulps, so called, and intended for the production of very white fiber of high alpha cellulose content and possessing characteristics which render it eminently suitable as a raw material for those manufactures where a substantially pure form of cellulose containing a very low percentage of objectionable impurities such as less-resistant celluloses, oxycelluloses, pentosans, lignin, and resin, is desired. Such fiber may be used as a substitute for cotton fiber in paper manufacture and in the preparation of cellulose derivatives such as nitrocellulose, cellulose acetate and cellulose xanthate, or cel-

lulose manufactures such as rayon, lacquers, celluloid, and the like.

Heretofore it has been difficult to refine an alkaline-digested pulp, such as kraft, to a substantially pure form of cellulose, owing to the high percentage of pentosans, lignin, and other coloring materials which are present in such pulp. Moreover, certain of the wood components are apparently transformed by alkaline digestion into dyestuffs which become so tenaciously fixed on the fiber that they are difficult to remove without degrading or injuring the fiber. It has been proposed to refine kraft pulp by first treating it with chlorine water, then redigesting it under pressure and at elevated temperature in an alkaline solution, and finally bleaching it. With such a process, however, if sufficient chlorine be used in the first step or sufficient bleach in the final step to produce fiber of high whiteness, it is found that such fiber has been permanently injured from both a physical and chemical standpoint.

In my application, Serial No. 73,193, filed December 4, 1925, I have described a process of refining alkaline-digested pulp. In accordance with that process, alkaline redigestion of the pulp is effected in a relatively concentrated alkaline solution at relatively low temperatures, for under such conditions it was found that the non-alpha cellulose components of such pulp, particularly the pentosans, were more effectively removed than in a relatively dilute solution at elevated temperatures. By first treating the pulp with chlorine water or hypochlorite, then redigesting such pulp in a relatively concentrated alkaline solution at relatively low temperatures, it was found possible to bleach the redigested pulp to a whiteness approximating that of ordinary bleached pulp, without material injury to the fiber, if a thoroughly cooked pulp is employed as a raw material. The treatments before and after alkaline redigestion, however, must be

carefully controlled, for if either is overdone in order to obtain the desired whiteness of fiber,—this being particularly likely when a normally cooked or undercooked alkaline-digested pulp is being treated,—the fiber is irreparably injured.

In practising the pulp-refining process utilizing the present invention, I may begin with a normally cooked or even an undercooked pulp, and treat such pulp before alkaline redigestion with a lignin-reactive reagent such as chlorine water, as described in my application for patent. But if the pulp is treated with a lignin-reactive reagent such as hypochlorite solution, or separately with chlorine water and hypochlorite solution, I now add sufficient free alkali to the hypochlorite solution to maintain it distinctly alkaline throughout the treatment. Under such conditions, degradation of the cellulose content of the pulp is prevented, as chlorine water is quite selective in its action upon lignin and coloring matter only, and alkaline hypochlorite solution acts quite similarly, as the free alkali apparently represses the intensity of oxidation sufficiently to prevent oxidation of the alpha cellulose which is less susceptible to oxidation.

Alkaline redigestion of the pulp may be effected after such treatment in a relatively concentrated alkaline solution at relatively low temperatures, as described in my application for patent, as under such conditions less-resistant celluloses, pentosans, together with reaction products of previous treatment, are readily reacted upon and dissolved from the pulp. The alkalinity of solution employed may be maintained at a point consistent with the product which it is desired to produce. For instance, where the final product is to be suitable both for papermaking and for conversion into cellulose derivatives, the concentration of alkali and temperature conditions should be such as not to effect mercerization, which impairs papermaking characteristics. When, however, the final product is to be employed for the manufacture of cellulose derivatives only, it may be preferable to maintain a concentration of alkali and temperature conditions which do effect mercerization, as under such conditions refinement of the pulp is more rapid and effective, and the mercerized fiber appears for some purposes to be better suited for conversion into derivatives. Preferably, where the alkaline solution contains compounds which do not react with an oxidant such as hypochlorite, I now add such an oxidant thereto, but in amount considerably less than that of the alkaline compounds. Thus, where a solution of caustic soda is employed for alkaline redigestion, it preferably also contains a certain amount of hypochlorite, as under such

conditions reaction upon lignin and other coloring matter in the pulp is promoted.

After alkaline redigestion, the pulp is bleached substantially to ultimate whiteness, but without physical or chemical injury to the fiber. In accordance with the process of this invention, the redigested pulp is bleached by a series of bleaching treatments, each of which treatments consists in subjecting the pulp to the action of bleach liquor containing relatively small quantities of hypochlorite and sufficient free alkali to maintain a distinctly alkaline condition during the treatment. If desired, after one treatment, the pulp may be digested in a relatively dilute alkaline solution at elevated temperature, as this effects a removal of lignin and other non-alpha cellulose components which consume hypochlorite, and thus makes possible a reduction of the hypochlorite necessary in reaching the desired whiteness.

The applicability of the process of my invention may best be appreciated by reference to specific examples of procedure, but it is to be understood that this invention is not limited to the precise quantities or proportions of the materials mentioned therein, as variations may be made, depending upon the raw pulp and the product which it is desired to produce.

The raw pulp to be refined may be produced by digesting chipped wood, e. g., spruce under pressure and at elevated temperature in an alkaline liquor such as the usual kraft liquor. In certain instances, it may be desirable to underdigest the chips to produce a high yield of long-fibered, strong pulp, as my refining process is not only applicable to a thoroughly digested pulp, but also to an underdigested pulp; but such latter pulp consumes more chemical in the treatments presently to be described. The pulp is, of course, washed and screened prior to being subjected to the refining process. The raw pulp may be first treated at a consistency of about 4% to 10% in chlorine water until the chlorine is practically all consumed, the percentage of chlorine necessary depending upon the purity of the pulp. In general, the treatment may be carried out in chlorine water containing 2% to 6% chlorine, based on pulp, for about 30 to 40 minutes. The chlorine may be added to the pulp all at once, or in doses so as to avoid a high chlorine concentration at any time. Where a fairly well-cooked kraft pulp containing about 3% to 5% chlorine is being treated, it is safe to add the chlorine all at once, if the treating temperature is maintained below 75° F. If desired, however, the chlorine may be added in doses, with intermediate washing of the pulp to remove acid reaction products which may injure the fiber. This treatment does not whiten the pulp, but

tends to deepen its color. In lieu of treating the pulp with chlorine water, particularly when such pulp is well cooked, I may treat it with hypochlorite solution containing sufficient alkali to maintain such solution distinctly alkaline throughout the treatment. For instance, the pulp may be treated with about 6% to 8% bleach containing about 1% to 2% caustic soda, based on pulp. Or a chlorine treatment followed by an alkaline hypochlorite treatment, or vice versa, preferably with an intermediate washing, may be employed. The chlorinating treatment and/or the alkaline hypochlorite treatment produces

- 5 reaction upon and removal of lignin and other non-alpha cellulose components of the pulp or renders them susceptible to solution by alkaline digestion.
- 10 The pulp is preferably washed substantially free of chemical and reaction products after the first treatment, and is redigested in a relatively concentrated alkaline solution at relatively low temperature. Thus the pulp may be redigested for about one hour at a
- 15 consistency of about 10% in 5% to 10% caustic soda solution, at a temperature of from 48° to 150° F., under which conditions the resulting fiber remains substantially unmercerized and is hence suitable both for cellulose derivative preparation and for papermaking. If the product is to be employed for cellulose derivative manufacture only, it may be preferable to employ a solution of greater than 10% strength, under such temperature
- 20 conditions as to produce partial or complete mercerization of the fiber. To this end, redigestion may be carried out at room temperatures or lower, for not only does low temperature favor mercerization, but with a given strength of caustic soda solution apparently effects a removal of pentosans, resins, and ligneous impurities, and accordingly an increase in alpha cellulose content more readily than higher temperature.

- 25 In lieu of using caustic soda solution for redigestion, I may use the so-called white liquor which is employed for kraft digestion. Such white liquor contains largely sodium hydroxide and sodium sulphide in solution, and usually has a sulphidity of from 20% to 40%. I may also use a liquor containing essentially only sodium sulphide, or one containing, in addition to sodium sulphide and/or caustic soda, a certain amount of sodium sulphite, which appears to react with the ligneous groups in the pulp. When the liquor contains chemicals other than sodium hydroxide, it is necessary that the concentration of such chemicals be higher than when sodium hydroxide is used, to effect a given refinement of the pulp, as chemicals such as sodium sulphide or sodium sulphite are not so highly active as sodium hydroxide. Thus, the usual kraft white liquor, to effect the same refinement as a liquor containing about 6% caustic

soda alone must contain about 8% caustic soda equivalent.

After alkaline digestion, the pulp is washed, preferably in a washer of the counter-current type, wherefrom unconsumed chemical may be recovered for reuse in preparing fresh alkaline liquor. The washed pulp is of high alpha cellulose content, and if the papermaking characteristics of the pulp have been preserved, paper made from such pulp is of much softer texture and of much higher tear resistance than that made from the original pulp. Thus, a kraft pulp having a strength of about 150 and a tear resistance of about 250, after alkaline redigestion has a strength of about 130 and a tear resistance of about 300 to 320. The drop in strength is doubtless traceable to the removal of pentosans, but this is not serious when a soft fiber of high tear resistance, which will serve as a rag fiber substitute, is desired. Its color, however, is usually not much lighter than that of the original pulp. When such pulp is subjected to bleaching, however, it is found that it bleaches much more readily than the original pulp. Thus, if it were attempted to bleach the original pulp substantially to ultimate whiteness, about 40% to 60% bleach, based on fiber, would be required, and severe degradation of the fiber would ensue. The alkaline-redigested pulp requires but from about 10% to 20% bleach to acquire the same degree of whiteness, but even such an amount of bleach, if employed as ordinarily, would materially impair the physical and chemical characteristics of the pulp. Thus, if the redigested pulp is bleached substantially to ultimate whiteness by the usual bleaching treatment, its strength falls to about 120 and its tear resistance to below 150. Soda solubility and copper number tests also indicate degradation of the cellulose content into oxycelluloses.

In accordance with my process, bleaching of the alkaline-digested fiber substantially to ultimate whiteness is effected without materially degrading the fiber. This is accomplished by subjecting the fiber to a series of alkaline bleaching treatments, preferably with alternating washings preferably with hot alkaline water. Washing may be effected in a washer of the countercurrent type, so that the wash water containing the active chemical of one treatment may be employed in a previous bleaching treatment, the last bleaching treatment being effected in fresh bleach liquor. The pulp may also be digested in an alkaline solution at elevated temperature between such bleaching treatments. Thus, the alkaline-redigested pulp may be treated at a consistency of from 6% to 10% in a solution containing 5% to 6% sodium or calcium hypochlorite and 1% caustic soda. The treatment may be carried out at tem-

peratures of about 70° to 100° F. for two to four hours, at the end of which time the bleach is practically all consumed. The pulp is then preferably washed and again treated in a solution of hypochlorite and caustic soda; then, if necessary, to a third and even a fourth treatment, until substantially ultimate whiteness has been reached. Preferably, any residual bleach in the finally washed, bleached fiber is neutralized with an anti-chlor such as sulphurous acid or sodium bisulphite.

It may be desirable to raise the alkali content of the bleaching liquor to 2% or 3%, based on pulp, particularly when the alkaline-digested pulp is rather difficult to bleach. In such case, a higher temperature is maintained during bleaching, to increase the rate of bleaching. Preferably, the treatment is commenced at relatively low temperature, and as the bleach is being consumed, the temperature is gradually raised to a final temperature of about 110° F. Or, as previously stated, it may be desirable to alkaline-digest the pulp at elevated temperature between bleaching treatments. As such alkaline digestion removes non-alpha cellulose components from the pulp, it makes possible the use of less bleach in subsequent bleaching treatments, or the elimination of one or more bleaching treatments. For instance, after the first bleaching treatment, the pulp may be digested for about one hour at about atmospheric boiling temperature in a 2% to 3% caustic soda solution, then washed before the succeeding bleaching treatment.

After bleaching, the fiber has reached substantially ultimate whiteness and not only compares favorably in chemical characteristics with a high grade alpha wood fiber prepared from sulphite pulp, but excels it in physical characteristics. Thus, the white fiber which I produce by the process of the present invention is usually stronger and possesses higher tear resistance than the alpha fiber produced from sulphite pulp.

What I claim is:

1. A process which comprises subjecting cellulose pulp to a series of distinctly alkaline hypochlorite bleaching treatments, one or more of said treatments commencing at relatively low temperature and gradually increasing during treatment to a final much higher temperature, alkalinity in said bleaching treatments being afforded by the presence of free alkali throughout each bleaching treatment.

2. A process which comprises subjecting cellulose pulp to a series of distinctly alkaline hypochlorite bleaching treatments, one or more of said treatments commencing at room temperature or lower and gradually increasing during treatment to a final temperature of about 110° F., alkalinity in said bleaching treatments being afforded by the

presence of free alkali throughout each bleaching treatment.

3. A process which comprises partially bleaching cellulose pulp in distinctly alkaline hypochlorite bleach liquor, digesting the partially bleached pulp at elevated temperature in dilute alkaline solution, and treating the digested pulp in a distinctly alkaline hypochlorite bleach liquor, alkalinity in said bleaching treatments being afforded by the presence of free alkali throughout each bleaching treatment.

4. A process which comprises redigesting previously digested pulp in alkaline solution and subjecting such redigested pulp to a series of independent, distinctly alkaline hypochlorite bleaching treatments, alkalinity in said bleaching treatments being afforded by the presence of free alkali throughout each bleaching treatment.

5. A process which comprises treating previously digested raw pulp with a chlorine-containing lignin-reactive reagent, redigesting the treated pulp in alkaline solution, and subjecting such redigested pulp to a series of independent, distinctly alkaline hypochlorite bleaching treatments, alkalinity in said bleaching treatments being afforded by the presence of free alkali throughout each bleaching treatment.

6. A process which comprises treating alkaline-digested wood pulp with a chlorine-containing lignin-reactive reagent, redigesting the treated pulp in alkaline solution, and subjecting such redigested pulp to a series of independent, distinctly alkaline hypochlorite bleaching treatments, alkalinity in said bleaching treatments being afforded by the presence of free alkali throughout each bleaching treatment.

7. A process which comprises treating alkaline-digested wood pulp with a chlorine-containing lignin-reactive reagent, redigesting the treated pulp in alkaline solution, and subjecting the redigested pulp to a series of alternating distinctly alkaline hypochlorite bleaching treatments and washings, alkalinity in said bleaching treatments being afforded by the presence of free alkali through each bleaching treatment.

8. A process which comprises treating alkaline-digested wood pulp with a chlorine-containing, lignin-reactive reagent, redigesting the treated pulp in a concentrated alkaline solution at low temperature, and subjecting such redigested pulp to a series of distinctly alkaline hypochlorite bleaching treatments, alkalinity in said bleaching treatments being afforded by the presence of free alkali throughout each bleaching treatment.

9. A process which comprises treating alkaline-digested wood pulp separately with chlorine water and with alkaline hypochlorite liquor, redigesting the treated pulp in alkaline solution, and subjecting such redi-

gested pulp to a series of distinctly alkaline hypochlorite bleaching treatments, alkalinity in said bleaching treatments being afforded by the presence of free alkali throughout each bleaching treatment.

10. A process which comprises treating alkaline-digested wood pulp with chlorine water, redigesting the treated pulp in a concentrated alkaline solution at about room temperature, and subjecting such redigested pulp to a series of distinctly alkaline hypochlorite bleaching treatments, alkalinity in said bleaching treatments being afforded by the presence of free alkali throughout each bleaching treatment.

11. A process which comprises treating alkaline-digested wood pulp with alkaline hypochlorite liquor, redigesting the treated pulp in alkaline solution, and subjecting such redigested pulp to a series of distinctly alkaline hypochlorite bleaching treatments, alkalinity in said bleaching treatments being afforded by the presence of free alkali throughout each bleaching treatment.

25. 12. A process which comprises treating alkaline-digested wood pulp with a chlorine-containing, lignin-reactive reagent, redigesting the treated pulp in a solution containing alkali and a much lower proportion of hypochlorite than alkali, and subjecting such redigested pulp to a series of distinctly alkaline hypochlorite bleaching treatments, alkalinity in said bleaching treatments being afforded by the presence of free alkali throughout each bleaching treatment.

13. A process which comprises treating alkaline-digested wood pulp with a chlorine-containing, lignin-reactive reagent, redigesting the treated pulp in a caustic soda solution under mercerizing conditions, and subjecting such redigested pulp to a series of distinctly alkaline hypochlorite bleaching treatments, alkalinity in said bleaching treatments being afforded by the presence of free alkali throughout each bleaching treatment.

40. 14. A process which comprises treating alkaline-digested wood pulp with a chlorine-containing, lignin-reactive reagent, redigesting the treated pulp in a concentrated alkaline solution at low temperature, and subjecting the redigested pulp to a series of alkaline hypochlorite bleaching treatments until the pulp has attained a white color, alkalinity in said bleaching treatments being afforded by the presence of free alkali throughout each bleaching treatment.

55. 15. A process which comprises treating alkaline-digested wood pulp with a chlorine-containing, lignin-reactive reagent, redigesting the treated pulp in alkaline solution, partially bleaching the redigested pulp in distinctly alkaline hypochlorite bleach liquor, digesting the partially bleached pulp at elevated temperature in a dilute alkaline solution, and again bleaching the pulp in a dis-

tinctly alkaline hypochlorite bleach liquor, alkalinity in said bleaching treatments being afforded by the presence of free alkali throughout each bleaching treatment.

16. A process which comprises digesting 70 pre-liberated kraft pulp in a substantially fresh kraft liquor of a composition similar to that in which fiber liberation was effected, and subjecting the digested product to a series of baths of distinctly alkaline hypo- 75 chlorite bleach liquor.

In testimony whereof I have affixed my signature.

GEORGE A. RICHTER.